

## UNITED STATES PATENT OFFICE

2,678,267

## METHOD OF MAKING AN ALLOY COMPRISING MAGNESIUM AND THORIUM

William P. Saunders, Midland, Mich., assignor to  
The Dow Chemical Company, Midland, Mich.,  
a corporation of Delaware

No Drawing. Application February 27, 1952,  
Serial No. 273,786

3 Claims. (Cl. 75—135)

1

The invention relates to magnesium alloys. It more particularly concerns a method of introducing thorium into melts of magnesium so as to form magnesium alloys containing thorium.

In attempting to produce alloys of magnesium and thorium by the conventional method of reacting a reducible thorium compound with molten magnesium in amount in excess of that corresponding to the stoichiometrical relationship  $\text{ThF}_4 + 2\text{Mg} = 2\text{MgF}_2 + \text{Th}$  whereby thorium is liberated in situ with the excess of the molten unoxidized magnesium, the difficulty arises that the alloying efficiency is low in that only a relatively small fraction (less than 10 per cent) of the thorium compound becomes alloyed with the unoxidized portion of the magnesium.

It is the principal object of the present invention to provide a method of forming alloys of magnesium with thorium by reacting a reducible thorium compound with molten magnesium whereby the efficiency of the alloying is increased. Other objects and advantages will appear as the description of the invention proceeds:

The invention is predicated upon the discovery that by using thorium tetrafluoride as the source of thorium and forming a melt of it with the chloride of one or both of the alkali metals potassium and sodium, a composition is obtained which yields magnesium-thorium alloys with increased efficiency of utilization of the thorium on subjecting the composition to the reducing action of molten magnesium in a proportion substantially in excess of that corresponding to the aforesaid stoichiometrical relationship as regards the thorium tetrafluoride content of the composition. The invention then consists of the improved method herein fully described and particularly pointed out in the claims.

In carrying out the invention, for each mole of thorium tetrafluoride used 3 to 7 moles of alkali metal chloride, as either or both potassium chloride and sodium chloride, are used therewith. One way of bringing these materials together to effect a reduction of the thorium tetrafluoride and bringing about alloying of the thorium liberated in the reduction with magnesium is as follows: Melt the requisite amount of alkali metal chloride in a suitable vessel, e. g. an iron or steel melting pot, and when the chloride is molten, add with stirring, the requisite amount of thorium tetrafluoride. The thorium tetrafluoride rapidly dissolves in the molten alkali metal chloride. The saline melt thus obtained is maintained at a temperature sufficient to melt magnesium, e. g., 1300° to 1600° F. and magnesium is added to the

5 saline melt in excess of the proportions indicated in the foregoing equation as regards the ratio of Mg to  $\text{ThF}_4$ . A small amount, e. g. 0.5 to 2 per cent of the weight of the magnesium, of a conventional magnesium foundry flux is preferably also added to protect the magnesium from attack by the atmosphere while the magnesium is molten and reacting with the  $\text{ThF}_4$  containing saline melt and becoming alloyed with thorium. 10 The resulting molten mixture is stirred for a short time, e. g., 2 to 20 minutes, during which the thorium tetrafluoride becomes reduced and the thorium liberated in the reduction alloys with the magnesium which is present in amount in excess of that required for the reduction. After stirring the molten mixture, it is allowed to settle for a few minutes, e. g., 5 minutes, and then the resulting floating metal regulus consisting of a magnesium-thorium alloy may be separated from 15 the resulting underlying saline sludge by decantation or otherwise.

The following examples are illustrative of the invention:

23

## EXAMPLE 1

15 pounds of potassium chloride is melted, and, while molten, 20 pounds of solid thorium tetrafluoride is added with stirring. The thorium tetrafluoride rapidly dissolves in the molten potassium chloride forming a slightly viscous saline melt containing 3.06 moles of KCl per mole of  $\text{ThF}_4$ . The molten saline melt is poured into a crucible containing 60 pounds of molten magnesium at 1350° F. and the contents of the crucible are stirred for 5 minutes. As the stirring proceeds, the temperature of the resulting mixture rises to about 1400° F., due to heat liberation as magnesium reduces the thorium compound to metallic thorium, a portion of which alloys with 30 the remaining magnesium. Stirring is continued 5 minutes more and then the mixture is left for 15 minutes at 1400° F., whereupon the thorium containing magnesium alloy segregates as a molten metal regulus floating upon a saline sludge. The floating alloy is decanted off and cast into an ingot. Its analysis shows a thorium content of 9.38 per cent. Had all the available thorium become alloyed with all the available magnesium, the resulting ingot would have contained 20.1 per cent of thorium by calculation. The alloying efficiency based upon this calculation is

$$\frac{9.38 \times 100}{20.1} = 47.6\%$$

## EXAMPLE 2

60 pounds of magnesium is melted under the

and 2. The following table sets forth the data obtained.

Table

| Test No. | Grams Mg. | Saline Melt            |                       | Moles Alkali Chloride per Mole ThF <sub>4</sub> | Percent Th in Resulting Alloy | Calculated Efficiency of Alloying |
|----------|-----------|------------------------|-----------------------|-------------------------------------------------|-------------------------------|-----------------------------------|
|          |           | Grams ThF <sub>4</sub> | Grams Alkali Chloride |                                                 |                               |                                   |
| 1        | 100       | 71                     | None                  | 0                                               | 2.3                           | 6.5                               |
| 2        | 100       | 71                     | 36 KCl                | 2.06                                            | 2.32                          | 6.7                               |
| 3        | 100       | 71                     | 54 KCl                | 3.10                                            | 9.36                          | 27.0                              |
| *4       | 100       | 71                     | 71 KCl                | 4.08                                            | 14.4                          | 41.0                              |
| 5        | 100       | 71                     | 88 KCl                | 4.88                                            | 15.85                         | 45.0                              |
| 6        | 100       | 71                     | 103 KCl               | 5.94                                            | 12.45                         | 35.5                              |
| 7        | 100       | 71                     | 142 KCl               | 8.14                                            | 6.14                          | 17.5                              |
| 8        | 100       | 71                     | 213 KCl               | 11.65                                           | 6.93                          | 20                                |
| 9        | 100       | 71                     | 54 NaCl               | 4.0                                             | 8.89                          | 25                                |
| 10       | 100       | 71                     | {36 KCl<br>26 NaCl}   | 4.07                                            | 13.79                         | 40                                |

\*Average of three tests.

protection of 1 pound of a magnesium foundry flux composed of 28 parts by weight of CaCl<sub>2</sub>, 57 parts of KCl, 12.5 parts of BaCl<sub>2</sub>, and 2.5 parts of CaF<sub>2</sub>. Thorium tetrafluoride and potassium chloride are fused together in the ratio of 4 moles of KCl per mole of ThF<sub>4</sub>. The resulting saline melt is solidified and broken into lumps about the size of a fist. 40 pounds of the lumps of the solidified saline melt of ThF<sub>4</sub> and KCl are added to the molten magnesium which is held at about 1400° F. and subjected to stirring for 20 minutes. During the stirring, an additional 5 pounds of magnesium foundry flux is added to protect the magnesium from attack by the atmosphere. The reaction which occurs, liberates thorium from the ThF<sub>4</sub>—KCl composition and a portion of the thorium alloys with the remaining magnesium. The stirred mixture is left for 10 minutes at 1400° F. to stratify. The resulting molten thorium containing magnesium alloy formed floats upon the resulting residue of saline sludge and is then decanted off and cast into an ingot. Its analysis shows a thorium content of 15 per cent. Had all the available thorium become alloyed with all the available magnesium, the resulting ingot would have contained 20.2 per cent of thorium by calculation. The alloying efficiency based upon this calculation is

$$\frac{100 \times 15}{20.2} = 75.7\%$$

A series of smaller tests were made which serve to indicate the effect of the mole ratio of alkali metal chloride to thorium tetrafluoride on the alloying efficiency. In these tests thorium tetrafluoride was dissolved in melts of alkali metal chloride to form saline melts having various mole ratios of alkali metal chloride to ThF<sub>4</sub>. Magnesium was then added to the saline melts which were stirred at temperatures of 1300° to 1600° F. The resulting mixtures of magnesium-thorium alloy and salines were settled. The alloys obtained were decanted off, cast into ingots, and analyzed for thorium. The efficiency of the alloying was calculated as in Examples 1

Referring to the table, it is manifest that the effect of increasing the ratio of the number of moles of alkali metal chloride to the number of moles of thorium tetrafluoride produces a sharp increase in alloying efficiency as the ratio exceeds 3. The efficiency of alloying reaches a peak at a ratio between about 4 and 6 then declines and levels off as the ratio exceeds about 7. A preferred operating ratio is about 4.5.

30 By the foregoing method, magnesium-thorium alloys containing various amounts of thorium, can be produced with increased efficiency of thorium utilization. For example, magnesium-thorium alloys containing from 0.1 to 35 per cent 35 of thorium or more can be made depending upon the amount of magnesium used relative to the thorium tetrafluoride. It is preferable to use at least 12 moles of magnesium per mole of thorium tetrafluoride although proportions as high as 40 1000 moles of magnesium per mole of thorium tetrafluoride may be used.

## I claim:

1. A method of making magnesium alloys containing thorium which comprises subjecting a saline melt of an alkali metal chloride selected from the group consisting of potassium chloride and sodium chloride, said saline melt containing thorium tetrafluoride in the ratio of between 3 and 7 moles of alkali metal chloride per mole of thorium tetrafluoride, to the reducing action of molten magnesium, the number of moles of magnesium being from 12 to 1000 times the number of moles of thorium tetrafluoride whereby metallic thorium liberated in the reduction becomes alloyed with magnesium.

2. The method according to claim 1 in which the alkali metal chloride is potassium chloride.

3. The method according to claim 1 in which the alkali metal chloride is sodium chloride.

## References Cited in the file of this patent

## UNITED STATES PATENTS

| Number    | Name         | Date          |
|-----------|--------------|---------------|
| 1,648,954 | Marden       | Nov. 15, 1927 |
| 2,497,537 | Emley et al. | Feb. 14, 1950 |
| 2,604,394 | Emley        | July 22, 1952 |